

Oct. 23, 1928.

1,688,645

E. E. NOVOTNY

PRINTING PLATE AND METHOD OF MAKING THE SAME

Filed Feb. 9, 1926

4 Sheets-Sheet 1

*Fig. 1*



*Fig. 2*



*Fig. 4*



*Fig. 5*



INVENTOR.  
*Emil E. Novotny*  
BY  
*Cavanaugh & James*  
ATTORNEYS.

Oct. 23, 1928.

1,688,645

E. E. NOVOTNY

PRINTING PLATE AND METHOD OF MAKING THE SAME

Filed Feb. 9, 1926

4 Sheets-Sheet 2



INVENTOR.

Emil E. Novotny  
BY  
Cavanaugh, James  
ATTORNEY.

Oct. 23, 1928.

1,688,645

E. E. NOVOTNY

PRINTING PLATE AND METHOD OF MAKING THE SAME

Filed Feb. 9, 1926

4 Sheets-Sheet 3

Fig. 6



INVENTOR.  
*Emil E. Novotny*  
BY  
*Cavanaugh & James*  
ATTORNEYS.

Oct. 23, 1928.

1,688,645

E. E. NOVOTNY

PRINTING PLATE AND METHOD OF MAKING THE SAME

Filed Feb. 9, 1926

4 Sheets-Sheet 4

Fig. 7



INVENTOR.  
Eduard E. Novotny  
BY  
Carrington & James  
ATTORNEYS.

## UNITED STATES PATENT OFFICE.

EMIL E. NOVOTNY, OF PHILADELPHIA, PENNSYLVANIA, ASSIGNOR TO JOHN STOG-  
DELL STOKES, OF SPRING VALLEY FARMS, HUNTINGTON VALLEY POST OFFICE,  
PENNSYLVANIA.

## PRINTING PLATE AND METHOD OF MAKING THE SAME.

Application filed February 9, 1926. Serial No. 87,111.

This invention relates to printing plates and the method of manufacturing the same.

My method of producing a printing plate is directed to the making of a structure which 5 lacks homogenous qualities. I wish to have a printing plate dissimilar from the usual metallic printing plates in use at the present time in order to attain a product which may be curved and leveled without the usual distortion. As for example, when a plate 10 which is first made in a flat condition is subsequently curved, considerable distortion takes place and there is an un-uniform elongation, resulting in great difficulty from a 15 dimensional and register standpoint. Furthermore, where the dimension in height to paper is either high or low in certain portions of the printing parts, it requires a more or less manual operation in order to bring 20 these to the proper level and then with more or less distortion to the surrounding areas. My aim, also, is to produce a printing plate 25 such as can be made by an inexperienced operator through the use of equipment which will utilize the inherent characteristics of a printing plate produced by my methods.

After long experimentation with various eutectic alloys in the form of foil and plastic metal, I have discovered that an alloy such 30 as, say, foundry type, monotype or other similar metals, even including mixtures of lead, tin and antimony, is most useful for my purpose. These alloys when applied to a suitable matrix by means of a metallic 35 spray properly adjusted form a structure which is not homogeneous and which apparently has had its particles combined through an alloy of lower melting point thrown out during the operation of the spray 40 ing. This results in exactly the conditions most desirable for a satisfactory form of commercial printing plate. In other words, the printing plate is formed from a bath of minute metallic particles which are still 45 in a somewhat plastic condition. These particles upon striking the surface, if the surface is properly prepared, are caused to deposit thereon, without rebounding therefrom, and form small, thin, scale-like portions. These portions are apparently oxidized 50 on their faces thus precluding the possibility of a solid, homogeneous welding action. In addition to this, I have observed, through tests which will be briefly described 55 later, the fact that these alloys evidently

throw out some of their heavier components while traveling under the influence of the spray. These components evidently promote the cementing of the particles, resulting in a relatively flexible structure upon heating at 60 a point well below the melting point of the alloy used.

Briefly, the test referred to consisted in the use of a plate made by my method wherein an alloy of foundry type metal was used, 65 having a melting point of about 650° F. This plate, when placed over a convex curved turtle heated to a temperature of approximately 400° F., took the curve of this turtle with a very slight amount of distortion and 70 fitted the turtle perfectly. Upon cooling, while supported in this manner, the plate retained its shape and was immediately available for printing purposes. A plate made by casting as in the stereotyping art, 75 using this same metal but producing a relatively homogeneous plate, was next tested. It was placed in the same position under the same conditions on the turtle before mentioned and the plate did not curve and it 80 would not curve of its own weight even after being heated to its melting point. Upon being heated to this high temperature it collapsed and the entire surface of the 85 printing plate was destroyed.

It can readily be seen that by using proper turtles suitable curves can be made and that there will be a minimum amount of stresses and strains on a curved plate of this kind. To emphasize the point still further, it might 90 be stated that both a commercial electrotyping and a commercial stereotype were substituted for the stereotype made of foundry metal and that a suitable curve could not be obtained without actually softening or melting 95 the entire body of such plate.

In leveling to a standard height to paper it is quite apparent that if we provide a suitable level base, place the plate face down on such base and heat to the point where 100 plasticity occurs, the plate will seek its own level without melting and without undue distortion. Of course, a slight amount of pressure is always desirable for both the leveling and curving operations, and therefore I provide a light pressure for this purpose.

For my purpose a matrix made of a plastic, waxy, fusible material is most suitable. The matrix material can be melted out 110

as is now practiced by the electrotyper and can be produced without undue stresses and strains on the original type matter. This waxy surface offers a special and peculiar advantage for the sprayed plate inasmuch as it is necessary to provide a suitable adherent surface which will hold the sprayed particles when they first are applied to such matrix surface. This is extremely impor-

10 tant inasmuch as otherwise the sprayed particles could not be evenly applied against such surface. A large portion of these would rebound upon impact, with the result that an even, highly polished reproduction would not result

15 In order to use a waxy matrix having a low softening point it is essential to provide a suitable cooling means either between subsequent applications of thin sprayed films

20 or preferably immediately following the area being sprayed in order not to unduly soften or distort the delicate matrix face. This I provide by means of an air nozzle which follows in the path of the spray nozzle

25 and removes with rapidity a large portion of the heat carried by the sprayed particles and by the heated air if it is used. I prefer at times to humidify the air in order that a greater and quicker cooling action may 30 then be secured.

It is quite desirable at times to reproduce work from matrices such as those of the lead mold type or such as those made in papier-mâché or other materials capable of standing

35 a higher temperature. This is true in the case of reproductions of fine etchings, etc., and a better resulting product is often obtained by the use of a matrix of this type where the electrotyping process is followed.

40 In following out my process it will be readily noted that a graphitic coating to insure conductivity need not be applied to the wax matrix and therefore the reproduction from wax will be fully up to that obtained from the lead mold.

45 Commercially, however, lead molded work is in demand and I provide a means for the use of non-waxy matrices by the application of a thin film of wax or Canada balsam to the surface of such matrices in order to provide a footing for the sprayed particles being applied thereon.

50 As these products are applied in a very thin solvent solution they do not affect the fidelity of the reproduction but are present in sufficient quantity to give the sprayed plate a fine, polished surface.

The wax matrix when used in my process is preferably supported by a suitable metallic base and at times by means of bearers along 60 the edges of such metallic base in order to obviate any possibility of the wax matrix curving or sagging during the application of the spray. This provision is an aid to the production of plates having the same dimensions of the printing parts in height to

paper as the original type matter and eliminates the possibility of matrix distorting, thereby stretching and giving dimensional errors throughout the printing area.

The use of alloys such as those mentioned 70 is very desirable where a plate having the plasticity before mentioned is wanted. It is, therefore, to be understood that I may make my plate of any sprayable material or metal which will be suitable for my purpose. For 75 certain cheap advertising plates it does not matter greatly whether there is a variation in height to paper and therefore it may be desirable to produce a plate using cheaper materials or using materials lighter in 80 weight, say, for example, aluminum. However, it will be found that even where these materials are used the method described by me of providing a matrix having an adherent film will be most suitable for this purpose 85 where a fine reproduction is desired.

A fine metallic spray is essential for the face forming portions of the printing plate. This is obtained by setting the air and metal outlet nozzles close together. A fine spray, 90 however, can be applied but slowly, and therefore, from a commercial standpoint, it is preferable to have more than one nozzle in order that a fine spray may first be applied and that this be followed by a coarse, quickly 95 applied body or backing portion. With the adjustable nozzle I employ, one nozzle can be used for both purposes as by operating upon a batch of matrices first to apply a facing coat; these matrices with their facing 100 coats may be operated upon later with the nozzle adjusted for coarse spray to secure a thick backing section more quickly. Likewise, a plurality of finely adjusted spray nozzles may be used, and if desirable a plurality of coarse spray nozzles can also be 105 used.

The fine spray portions may be composed of different alloys or, for that matter, formed 110 of a tough wearing material such as, for example, aluminum, copper or nickel, and this may subsequently be backed with a fine spray and a coarse spray application, or, in some instances, the fine spray backing may be omitted.

The application of tougher films to the face may be done by subjecting the sprayed plate to a subsequent electrolytic deposit. This harder face backed up with a non-homogeneous metal offers advantages such as are not present in the solid homogeneous metal plates when it comes to a leveling and curving operation. The face section is hard and not readily damaged through pressure 120 against a level surface plate, whereas the body portion when heated well below its melting point will assume a plastic condition without melting and without lateral elongation or distortion. This protection 125 of a harder face, whether applied by a spray 130

or subsequently by means of an electrolytic deposit, while being useful in giving longer wear to the finished printing plate also helps to prevent the marring of a delicately ornamented printing surface.

The printing plates made entirely of type founder's metal having at first a fine sprayed facing section backed up with a coarse sprayed backing section were given an endurance test in actual high grade printing on coated stock. These plates have shown a production under actual printing conditions of over 300,000 high grade impressions. This test shows conclusively that these plates are capable of standing long runs. It is considered a very good production to secure 250,000 impressions from a nickel faced electrotype.

In the accompanying drawings—

20 Fig. 1 shows a cross sectional view of a wax matrix supported in a suitable pan.

Fig. 2 shows a cross sectional view of a lead matrix having a wax coating applied thereon.

25 Fig. 3 is a perspective view showing the apparatus in position to be employed in spraying against the face of a suitable matrix.

Fig. 4 is a cross sectional view showing 30 a printing plate made by my method wherein a fine facing spray is first applied and being subsequently backed with a coarser sprayed body forming section.

Fig. 5 is a cross sectional view of a modified form of printing plate similar to that shown in Fig. 4 with the exception, however, that a harder face coating is applied either by means of a spray or by a subsequent electrolytic deposit.

40 Fig. 6 is a perspective view showing the apparatus and plate in position for leveling.

Fig. 7 is a perspective view showing the apparatus used and printing plate in position thereon after having been curved.

45 In operating my invention I produce a suitable matrix as shown in Fig. 1 and indicated as an entirety by M. This matrix blank is first formed by pouring a suitable wax-like composition 1 into the pan P. The impression is taken in this wax in any well known manner, the face forming portion being indicated at 2.

50 Another form of matrix used for this purpose is made of any high melting point material such as the lead mold or matrix shown in Fig. 2 and indicated as an entirety by M. At 2, I indicate the face forming portion of such matrix, and the application of the adherent or waxy material at 3. This waxy material may consist of a weak solution of say beeswax or Canada balsam, a suitable solvent being used.

60 Fig. 3 shows the apparatus in its simplest form, illustrating the method of operating upon the matrix M which is supported upon

a suitable movable carriage C, traveling upon tracks T. This carriage gives both longitudinal and transverse motion by means of the arms 5 and 6. This provides a suitable means for maintaining a relatively fixed distance between the matrix M and the metal spray nozzle S.

The metal is contained in the furnace or melting pot F which is heated by suitable means as by the electrical heating unit terminating in the leads indicated at 7. When foundry type metal is used this has a melting point of approximately 650° F. and it is preferably heated to a temperature not to exceed 850° F. The molten metal is controlled by means of a plug valve indicated by the screw and knob terminus thereof at 8. The metal issues from the nozzle S, the nozzle being sufficiently heated by the excess heat carried by the metal and is vaporized into a fine spray by the air nozzle A which is made adjustable by means of the adjustment device indicated as an entirety at 9, a supply of heated air being conducted thereto by pipe 10, the heating of the air being accomplished through the use of the heater shown as an entirety at H consisting of coils 11, operating in the zone of a suitable source of heat as at 12. The nozzle S I find should have an opening not greatly exceeding a diameter of .020" whereas the nozzle A for the air is considerably larger but preferably should not greatly exceed a diameter of .070".

It will be noted by reference to Fig. 3, that molten metal flows from the melting pot by gravity, and therefore the liability of the particles striking the matrix and rebounding, or being welded together in a homogeneous mass, as would be the case with removing the molten metal from the pot under pressure, is avoided.

A suitable cooling means is provided as by means of the cold air nozzle A' connected to the pipe 13, and if at times a small amount of water is useful this is provided by means of the water nozzle W terminating in the pipe 14.

The spraying apparatus in Fig. 3 is suitably hooded as by means of the hood conventionally shown at H' terminating in a suction fan opening indicated at 15 which may be at either the top or the bottom of this hooded device, suitable doors being provided at 16. The lower section of this hood H' serves to retain any dust particles which may settle and which may not be removed through the opening 15 by means of the fan and cyclone receptacle (not shown), this cyclone receptacle serving to deposit any metallic particles which may be carried over by the air in a manner already well known.

In Fig. 4 I show the completed plate indicated as an entirety by P'. This printing plate consists of a facing of finer sprayed

particles indicated at 17, forming the highly polished face 18 and the coarser sprayed or less homogeneous particles forming the backing indicated at 19. The back portion of 5 such plate has been roughly shaved and is indicated at 20.

Fig. 5 indicates a printing plate very similar to that shown in Fig. 4 wherein the printing plate again is indicated as an entirety by P'. The printing face indicated at 18' consists of a tougher metal which may be either applied as a spray or which may be applied subsequently as an electrolytic coating. This may be followed optionally 10 with the finer sprayed facing section 17 and the coarser sprayed backing section 19, the back thereof being again shown at 20.

In Fig. 6 I show the leveling apparatus indicated as an entirety by L supported on a 20 suitable stand or base. This leveling device L consists of a level surface plate section S' which is heated as conventionally shown by the gas cock at 21. As stated previously, this base is so heated that the plate will 25 quickly assume a temperature of approximately 400 to 500° F., the plate lying with its face 18 against the polished surface plate S', and proper pressure is applied as by means of the screw 22 operating against the platen 30 28. A suitable resilient blanket (not shown) is preferably placed between the back of the printing plate 20 and the lower section of the pressure platen 23, in order that a light pressure may be applied and that any irregularities may be taken up in this blanket. A suitable cooling means is provided as by 35 means of the inlet hole 24 and outlet hole 25, for the admission of cooling water in order that the plate may be quickly cooled 40 by circulating cooling water in a properly cored cooling plate.

In Fig. 7 I show an apparatus conventionally shown for the purpose of curving my sprayed plates. This apparatus is indicated as an entirety by B which is supported 45 on a suitable base. This curving apparatus consists essentially of a heating base indicated as an entirety as S', having a polished curved base section 18' suitably heated as 50 conventionally shown by the gas cock 21. Pressure is applied by means of the screw arrangement 22 operating against the concave polished platen 23 against the face of the printing plate 18, the back of which is indicated by 20. Suitable cooling facilities 55 are again provided as for the leveling apparatus by means of the openings to the cored out section of the base S' wherein 24 indicates the inlet for cooling water and 25 an opening for a suitable outlet. The plate 60 is placed face up upon the heated platen S' until the desired temperature is reached. This for foundry type metal will be between 400 and 500° F. It will be found that the 65 plate has assumed its curved form and that

a slight pressure from the platen 23 will cause the plate to assume the curve provided for by the concave section 23 and convex section 18'. For some purposes a resilient 70 blanket (not shown) may be interposed between the back of the plate 20 and the convex section 18' in order that irregularities may be taken up.

It will, of course, be understood that instead of producing ordinary relief plates 75 by this process, I may produce intaglio plates by the use of suitable originals or by means or ordinary expedients such as, for example, inversion.

While I have herein shown and described 80 certain preferred embodiments of my invention, I wish it to be understood that I do not confine myself to all of the precise details herein set forth, as modifications and variations may be made without departing from 85 the spirit of the invention or exceeding the scope of the appended claims.

Although I have stated in the preceding portion of the specification that the air nozzle A is furnished with a supply of 90 heated air by being conducted through pipe 10 and through heater coils 11, it should be understood that in certain cases it may be possible to dispense with the heating of this air, in which case the source of heat 12 may 95 be merely omitted. Using certain metals or alloys capable of absorbing a certain amount of superheat, this may be sufficient to produce a fair grade of sprayed work 100 without the use of the hot, dry air. The dimensions for the nozzles S and A should be provided with suitable openings to take care of the type of metal used. Where the dimensions given are for type founders metal, other alloys or metals may require 105 certain variations in these dimensions. However, it will be found preferable in all cases to have the nozzle A of larger diameter than the nozzle S.

What I claim is—

1. A printing plate having a non-homogeneous type-forming face of sprayed metallic particles.

2. A printing plate having a non-homogeneous type-forming face of sprayed metallic particles and a suitable support or 115 backing for the face portion.

3. A printing plate having a non-homogeneous type-forming face portion of sprayed metallic particles and a backing portion also composed of sprayed metallic particles.

4. A printing plate having a non-homogeneous type-forming face portion of sprayed particles of a metallic alloy, and a backing 120 portion for the face portion.

5. A printing plate having a porous non-homogeneous printing face of fine sprayed metallic particles, and a backing portion therefor of coarser sprayed metallic particles.

6. A printing plate composed of non-homogeneous sprayed metallic particles having a printing face surfaced with a film of hard, wear-resisting metal.

7. The herein described method of making a printing plate which comprises subjecting a gravity flowing stream of molten metal to the action of an air blast to impinge the metal in the form of a finely divided spray against the reproducing face of a printing plate matrix, and continuing such application until a printing plate of predetermined thickness is formed.

8. The herein described method of making a printing plate which consists in depositing upon the reproduction face of a printing plate matrix, successive films of molten metal applied in the form of a spray, said metal being so constituted that the printing plate may be flexed when heated below the melting point of the metal.

9. The herein described method of making a printing plate which consists in subjecting a suitable matrix to a spray of metallic particles to produce a relatively thin non-homogeneous metallic deposit forming a printing face, and then making a subsequent application of sprayed metal until a plate of suitable thickness is produced.

10. The herein described method of making a printing plate which consists in subjecting a suitable matrix to a spray of metallic particles to produce a relatively thin non-homogeneous metallic deposit, cooling said deposit, and then making subsequent applications of sprayed metal until a non-homogeneous metallic plate of suitable thickness is produced.

11. The herein described method of making a printing plate which consists in spraying molten metal against a suitable matrix to produce a non-homogeneous metallic printing plate face portion, and then making subsequent applications of sprayed metallic particles to build up a backing portion of suitable thickness.

12. The herein described method of mak-

ing a printing plate which consists in exposing a suitable matrix in the zone of a metallic spray to form a non-homogeneous 50 metallic printing face and body portion, and subsequently depositing, electrolytically, a tough wear-resisting metallic film on the printing face of said plate.

13. The herein described method of making a printing plate which consists in depositing upon the matrix, having its reproducing face coated with a wax-like substance, molten metal in the form of a spray to form a non-homogeneous printing plate 60 face, making subsequent applications of the metallic spray to build up a printing plate body of suitable thickness, and cooling the metal of the plate between applications.

14. The herewith described method of 65 making a printing plate which consists in exposing a portion of a suitable matrix in the zone of a metallic spray, applying a thin metallic coating while moving the metal coated matrix portion toward the zone of a 70 cool air nozzle to quickly cool the metallic film previously applied.

15. The herewith described method of making a printing plate which consists in exposing a portion of a suitable matrix 75 in the zone of a metallic spray, applying a thin metallic coating on a portion of the matrix or printing plate being formed while simultaneously moving the coated portion in the direction of the cooling zone of cool 80 moist air to quickly cool the metallic film previously applied.

16. The herein described method of making a printing plate which consists in spraying heated metallic particles against a suitable matrix to form the printing plate while employing heated air to prevent the premature chilling of the metallic particles during the spraying operation.

Signed at Philadelphia, in the county of 90 Philadelphia, and State of Pennsylvania this 5th day of February, A. D. 1926.

EMIL E. NOVOTNY.